

## 1

2,826,506

**COMPOSITION FOR TREATING FIBROUS MATERIALS**

Ralf B. Trusler, Dayton, Ohio, assignor to The Davies-Young Soap Company, Dayton, Ohio

No Drawing. Application December 5, 1952  
Serial No. 324,420

2 Claims. (Cl. 106—208)

This invention relates to the treatment of fibrous materials and, more particularly, to rendering fibrous materials electro-conductive while simultaneously applying a sizing agent to them.

Various types of fibers, including both natural and artificial synthetic fibers, and yarns, fabrics and the like comprising them, are easily electrified, even by the simple process of working the fibers into yarns, during fabricating the yarns, as by knitting or weaving, or by merely handling the fabrics.

In working up loose masses of discontinuous or staple fibers to a spun yarn on conventional yarn-spinning equipment, the combing and/or carding of the fibers, formation of a sliver or roving, and passage of the bundle of fibers through the drafting rollers are complicated by the tendency of the fibers to become electrified by friction and to be attracted to and adhere to the metal parts of the apparatus in the electrified state. Likewise, in knitting various yarns, such as nylon yarns, smooth knitting is hampered by the tendency of the yarns to become electrified.

Fabrics comprising fibers which are not electro-conductive are attracted to oppositely charged and to neutral objects, to which they tend to cling tenaciously. For example, a woolen sweater or dress becomes charged with static electricity during the act of dressing and undressing. A nylon garment has been found to be highly electrified after it is drawn across woolen blanket or similar kind of fabric. Similarly, garments which have been laundered or dry-cleaned and placed in a hamper attain some degree of electrification through the mere act of separating one garment from others in the hamper.

Clothing in a state of static electrification attracts particles of dust and soil which have a dulling effect on the appearance of the fabric. Women's skirts and men's trousers, when electrified, are attracted to furniture such as chairs and sofas and make a dynamic contact with the seat of the chair, with the result that more soil is wiped off on the fabric than would wipe off if the fabric were not charged. Dust soil and other foreign matter, for instance cat and dog hairs, thus picked up by electrostatically charged clothing are firmly adherent to the clothing and difficult to remove therefrom by brushing.

The problem of rendering fibrous materials resistant to the accumulation of electrostatic charges is complicated by the fact that, in most instances, it is also desirable to apply a sizing agent to the fibrous material for the purpose of improving the workability or processability of the fibers or yarns, or for stiffening and improving the "hand" or "feel" of the fabric.

It is not feasible to size the fibrous material, for example, a fabric, and render the same electro-conductive by a two-step method involving first dipping the fabric into a solution of one of the known or conventional sizing agents, drying the fabric, and subsequently dipping the fabric into a solution of one of the known anti-static agents, or by reversing the order of application of the solutions, because of the danger that the solvent used as

## 2

vehicle for the agent applied in the second treatment will dissolve out the agent applied in the first treatment when the fabric is later dipped into the solution used in the second stage of the two-step procedure.

5 Likewise, it is not practical to size the fibrous material and render it electro-conductive by a two-stage method in which the fabric or the like is sprayed first with a solution of one of the conditioning agents, either a sizing agent or an anti-static agent, and then with a solution of the other of those agents. Such a method requires two drying operations and, if aqueous solutions of the agents are used, the method is limited to the treatment of washable fabrics since, if fabrics which are not washable are treated in that way, they are subject to damage by excessive exposure to water.

10 Furthermore, if an aqueous solution of an anti-static agent is sprayed on a fabric carrying a water-soluble size, or if the applications are carried out in reverse order, the water applied with the second spray tends to flush out the water-soluble agent deposited on the fabric by the first spray. The same problem arises if the respective agents are applied in a dry-cleaning solvent.

15 One object of the present invention is to provide a method for sizing fibrous material and rendering it electro-conductive in a single treatment.

20 Another object is to provide a novel treating composition for fibrous materials comprising a homogeneous stable dispersion or solution of a mixture of a sizing agent and an anti-static agent.

25 A further object is to provide a method of simultaneously sizing fibrous material and rendering it electro-conductive which may be accomplished by a wet process in which the fibrous material is wet with water and the mixed sizing and anti-static agents are water-borne, or by a dry process in which the fibrous material is treated with a non-aqueous liquid such as dry-cleaners' naphtha having the sizing and anti-static agents incorporated therein.

30 Other objects and advantages of the invention will appear hereinafter.

35 In accordance with this invention, fibrous materials are simultaneously sized and rendered resistant to the accumulation of static charges by treating the material with an aqueous or non-aqueous dispersion, including solution, comprising a sizing agent and an anti-static agent, removing excess treating solution, if that is necessary, and drying the fibrous material.

40 As useful water-soluble or water-dispersible sizing agents there may be mentioned such natural, vegetable products as gum karaya, gum arabic and starch, as well as chemically produced substances such as glue, prepared casein, polyvinyl alcohols and carboxymethyl cellulose salts. Sizing agents which are soluble or dispersible in dry-cleaning solvents and suitable for treating the fibrous materials by the dry method using dry-cleaning solvents as vehicles, include copal gums, ester gums, phenol formaldehyde resins and silicone resins. The "sizing" agents mentioned are all normally solid or highly viscous, non-oily materials which impart a gain in stiffness to the material treated.

45 The anti-static agent may be a humectant or hygroscopic agent which increases the moisture pick-up and retention capacity of the fibrous material so that, in equilibrium with the atmosphere, it retains sufficient moisture to render it electro-conductive. Or the anti-static agent may be a soluble or dispersible organic or inorganic electrolyte which renders the fibrous material electro-conductive even at low atmospheric relative humidity.

50 A fairly wide variety of sizing agents and anti-static agents may be used in admixture. However, to accomplish the objectives of this invention and in order effec-

tively to render the fibrous material electro-conductive so that static charges are nullified or immediately discharged, while simultaneously conditioning and sizing the material, certain criteria must be observed in selecting the sizing agent and anti-static agent to be used in combination. Thus, it is essential to select sizing agents and anti-static agents which are mutually compatible in the aqueous or non-aqueous vehicle in which they are to be applied to the fibrous material.

After considerable research and experimental work on this problem, I have established that, in general, the anti-static agent and sizing agent may be selected on the basis of their mutual compatibility in the selected "wet" or "dry" vehicle to yield clear, essentially transparent, homogeneous and stable solutions or dispersions when they are used in certain predetermined concentrations. It is found that any sizing agent which is soluble or dispersible in the selected vehicle and which, in a concentration between 0.001% and 40% by weight, based on the total solids weight of the composition, remains dissolved or dispersed in the vehicle in the presence of between 0.001% and 40% of the anti-static agent, may be used. Conversely, any anti-static agent which is soluble or dispersible in the selected vehicle and, in concentrations between 0.001% and 40% by weight, based on the total solids weight of the composition, remains dissolved or dispersed in the vehicle in the presence of 0.001% to 40% of the selected sizing agent, and may be used.

By "total solids weight" as used herein is meant the combined weights of the sizing agent and the anti-static agent.

Various combinations of anti-static agents and sizing agents which may be used are exemplified in the examples given below. Other combinations can be arrived at empirically, using the stated criteria.

Concentrated solutions or dispersions of the mixed anti-static and sizing agents may be prepared initially and stored, to be diluted to a less concentrated condition at a subsequent time, such as immediately prior to application to the fibrous material. Thus concentrates containing 5% up to the compatible limits of each of the respective agents may be prepared as clear, essentially transparent solutions or dispersions which may be stored for indefinite periods without precipitation of the sizing or anti-static agent, and the concentrates may be later diluted with additional amounts of water or of a dry-cleaning solvent, as may be appropriate. In both the concentrated and the diluted condition, the compositions are homogeneous and stable since the agents are selected so that under normal conditions of storage and use, neither active agent of the composition is precipitated by the other.

The fibrous material may comprise or consist of natural fibers such as cotton and wool, or it may comprise or consist of artificial or synthetic fibers made from such fiber-forming materials as regenerated cellulose; cellulose esters such as cellulose acetate; cellulose ethers of the type of carboxymethyl cellulose and hydroxyethyl cellulose in which the ratio of ether groups to anhydroglucose units encompasses the range including the water-soluble ethers, the water-insoluble, alkali-soluble ethers and the organic solvent-soluble ethers; cellulose thiourethanes and polyamides of the nylon type (e. g. polymeric condensates of dibasic acids and diamines).

The fibrous material may also comprise or consist of fibers of polyesters of the "Dacron" type (e. g. polymeric condensates of terephthalic acid and glycols); polyethylene; polytrifluorochlorethylene; polytetrafluoroethylene; copolymers of vinyl chloride and vinyl acetate ("Vinyon"); copolymers of acrylonitrile and vinyl chloride ("Vinyon N"); polycarboanhydrides; fiber-forming polyvinylchloride; fiber-forming polyvinylidene chloride; copolymers of vinylidene chloride and vinyl chloride ("Saron"); polyacrylonitrile; copolymers of acrylonitrile with at least one other monoethylerically unsaturated

monomer copolymerizable with acrylonitrile, including binary copolymers of acrylonitrile with vinyl acetate, methacrylonitrile, or an acid dye-receptive monomer of the type of vinylimidazoles and vinylpyridines such as 5 2-vinylpyridine or 2-methyl-5-vinylpyridine and containing at least 70% of acrylonitrile in the polymer molecule, as well as ternary copolymers containing, in addition to polymerized acrylonitrile, two other, different monomers, particularly terpolymers containing, in the polymer molecule, in addition to a minor amount of a third monomer such as methacrylonitrile, at least 70% of acrylonitrile and at least 2% of a monomer receptive to dyestuff, such as a vinylpyridine or a vinylimidazole.

10 The fibrous materials may also comprise or consist of spinnable blends of two or more acrylonitrile polymers such as a blend of a base polymer which may be polyacrylonitrile or a copolymer of acrylonitrile and, for instance, vinyl acetate, high in acrylonitrile, i. e., containing at least 90%, preferably from 92-98%, of acrylonitrile 15 in the polymer molecule, with a modifying acid dye-receptive copolymer of acrylonitrile and a vinylpyridine containing between 30 and 70% by weight of acrylonitrile in the molecule. Such a blend may consist of, for example, 20 80 to 95 parts by weight of a base polymer of 97% acrylonitrile and 3% vinyl acetate with from 2 to 20 parts by weight of a modifying, acid dye-receptive copolymer of 50% acrylonitriles and 50% of a vinylpyridine.

25 The fibrous material may be in any form. For example, loose masses of discontinuous or staple fibers may 30 be sized and rendered electro-conductive preparatory to being spun into a yarn, or assembled in a felt-like structure in which the fibers are either arrayed in a substantially parallelized condition or in random arrangement, by spraying the fiber mass with a solution or dispersion 35 containing the compatible sizing and anti-static agents, or by placing the masses of fibers on a foraminous conveyor and drawing them through the solution or dispersion.

30 The fibers may be in a crimped condition imposed mechanically or resulting from the inherent character of the 40 fibers and the manner in which they have been handled. Thus, the fibers may be obtained from filaments formed of two different fiber-forming materials having different characteristics rendering the filaments reversibly convertible between a substantially straight condition and a 45 crimped condition, the discontinuous fibers being in the crimped condition.

45 The short fibers may be obtained from conjugated filaments comprising two components, each comprising a different thermoplastic fiber-forming material arranged in 50 side-by-side relationship, one of the thermoplastic components being more heat-shrinkable than the other, so that on heating in a relaxed condition to the shrinkage temperature for the more readily shrinkable component, that component shrinks causing buckling of the less heat-sensitive component, and crimping of the conjugated filament as a whole. Such crimped filaments, after setting thereof in the crimped state by cooling, may be cut or otherwise reduced to short fibers, which are then sized and made electro-conductive by treatment with the homogeneous composition containing the sizing and anti-static agents.

55 Continuous filaments or yarns may be treated as running lengths, in the form of skeins or hanks, or after collection in wound package form, as on a bobbin, spool or pirn, or in the form of an unsupported wound filamentary package or "cake," by passing the homogeneous treating agent through the windings of the package.

60 The treatment may be performed in a field of sound waves having a frequency of a thousand to a million 70 or more cycles per second, whereby the treating composition is impelled through the windings and uniform distribution of the treating composition on the yarn is facilitated. Continuous filaments or yarns may be gathered into a bundle or tow of high total denier, and treated with the homogeneous solution or dispersion of

the sizing and anti-static agents and dried, as they proceed to a subsequent collecting or disrupting zone, for instance a zone in which they are reduced to discontinuous lengths by breaking or cutting.

The filaments or yarns of the bundle may be crimped prior to application of the solution or dispersion of the mixed sizing and anti-static agents, after such treatment, or intermediately of the stage at which they are treated with the homogeneous solution or dispersion and the stage at which they are reduced to short lengths.

For instance, when the filaments or yarns making up the bundle or tow comprise thermoplastic fiber-forming material, the bundle may be directed in a predetermined path along which it is treated with the sizing and anti-static solution or dispersion, dried as by subjecting it to the action of warm air currents, passed into a chamber equipped with a steam injector and in which the filaments or yarns are forced to pile up and are crimped by back-pressure under the influence of the steam, and thence to a collecting or cutting zone.

The yarns, such as nylon yarns, may be treated with the solution or dispersion containing the sizing agent and the anti-static agent, and dried, as they are fed to the needles of a knitting machine.

Fabricated structures, which may be knitted, woven, netted, braided, etc., including articles of clothing, draperies, blankets, spreads, needled felts and felt-like products of the kind frequently described as "non-woven fabrics," i. e., products comprising matted or intermingled fibers associated together to form a compact material obtained without benefit of spinning or weaving, leather and paper, may be sized and rendered electro-conductive in a single operation by treatment in any suitable way, as by spraying, dipping, by passage in contact with a brush or the like rotating in a bath of the treating solution and arranged to transfer the solution to the fibrous material, and then dried at ordinary temperature or at elevated temperature below the temperature at which the fibers would be damaged.

Fabrics and articles of clothing may be sized and rendered electro-conductive in the course of finishing them for marketing. They may be restored to their initial sized, electro-conductive condition after laundering or dry-cleaning, by treatment with the homogeneous solution or dispersion of the mixed sizing and anti-static agents either as a step in the laundering or dry-cleaning process or as an after-treatment of the laundered or dry-cleaned goods.

In preparing the homogeneous compositions of the invention, the selected sizing agent may be dissolved or dispersed in water or the dry-cleaning solvent, with heating and stirring as may be required to effect the dissolution or fine dispersion, and thereafter the anti-static agent compatible with the sizing agent in concentrations of 0.001% to 40% may be dissolved or dispersed in the solution of the sizing agent. As already noted, the product obtained initially may be highly concentrated, containing amounts of the sizing and anti-static agent in the upper limits of the ranges stated, and diluted as desired at a later time.

In the following examples, specific embodiments of the invention are given and representative mixtures of sizing agents and anti-static agents which may be used are set forth. It will be understood that these examples are given by way of illustration only, and that the invention is not limited to the particular mixtures of anti-static and sizing agents shown therein.

#### Example I

A concentrated sizing and anti-static composition was prepared by dissolving 50 grams of gum arabic in 450 grams of boiling water, adding 5.0 grams of the anti-static agent, alkyl ( $C_9$  to  $C_{12}$ ) [alkyl ( $C_9$  to  $C_{12}$ )-butyl-methyl]-trimethyl-ammonium chloride having the formula



5 to the solution, and stirring mixture until the anti-static agent was dissolved.

Fifty grams of the concentrate were stirred into 250 grams of water to obtain a diluted solution suitable for spraying.

10 A piece of cotton lace was sprayed with the solution, and a piece of nylon netting was immersed therein. The fabrics were then dried and pressed. They were found to have acquired an increased stiffness desirable for decorative and dressmaking purposes. When the dried, pressed pieces of fabric were brushed and stroked with a smooth, varnished wood stick, they did not become electrified and exhibited no attraction for particles of dust or other foreign matter.

20

#### Example II

One hundred grams of gum arabic were dissolved, with stirring, in 895 grams of water, and 5 grams of a di-polyalkanolalkylamine anti-static agent were dissolved in the gum solution.

25 Pieces of cotton and nylon cloth were treated with this solution as in Example I. After removing excess treating liquid and drying and pressing the cloths, they were found to have acquired a stiff, crisp "hand" and to be resistant to the accumulation of static charges.

30 In comparison, similar pieces of cloth which were sprayed with the gum solution, without the addition of the nitrogenous anti-static compound, were stiffened but were readily electrified by friction.

NOTE.—The di-polyalkanol alkylamine used in this example was of the type having the structural formula:



40 where R is a methyl or ethyl radical and x and y are each in integer from 1 to 5.

#### Example III

45 Ten grams of laundry starch were boiled in 400 grams of water, and 40 grams of calcium chloride were added.

A piece of nylon cloth was immersed in the solution, wrung to remove the excess, dried and pressed.

48 This treatment imparted a pleasing stiffness to the fabric and rendered it electro-conductive.

#### Example IV

50 Twenty grams of a water-soluble polyvinyl alcohol were stirred into 980 grams of boiling water. The solution thus obtained was divided into two equal portions. One of these portions was diluted with 495 grams of water containing 1.0 gram of urea to obtain a treating solution A. A piece of silk cloth immersed in the solution A, squeezed to remove the excess liquid, dried and pressed, was found to have acquired a perceptible stiffness and to be resistant to electrification when it was subjected to friction by rubbing it across a clean glass plate.

55 A similar fabric immersed in the other portion of the initial solution acquired a definite stiffness but was easily electrified by rubbing across the glass plate.

#### Example V

60 An additional 3.0 grams of urea were added to a solution A as in Example IV. A piece of silk immersed in the solution, squeezed, dried and pressed, did not exhibit any visible change in texture or color as the result of treatment with the solution containing the increased proportion of urea, and was even more resistant to electrification than the fabric treated in solution A containing the lesser amount of urea.

7  
*Example VI*

Twenty-five grams of the commercially available resin "ST-137X" (phenol formaldehyde resin precondensate) were dissolved in 470 grams of toluene. Five grams of dibutyl acid phosphate were then dissolved in the solution. A 12" square piece of silk dress goods was wet with the solution and dried. It was sized satisfactorily and also resisted electrification.

In contrast, when a piece of silk as above was immersed in the toluene solution of the phenol-formaldehyde resin in the absence of the dibutyl acid phosphate, the fabric was less resistant to electrification than before the treatment with the solution.

8  
*Example VII*

Twenty grams of the commercially available resin "Piccolyte S-85" (a terpene resin) were dissolved in 475 grams of mineral spirits. Two grams of the quaternary ammonium anti-static compound [alkyl (C<sub>9</sub> to C<sub>15</sub>)-tolylmethyl]-trimethyl ammonium chloride having the formula



were then dissolved in the solution of the terpene resin size. A piece of white poplin was wet with the solution, and dried. It had an attractive, crisp "feel" and was found to be resistant to electrification when struck with a rod formed of a methyl methacrylate resin.

9  
*Example VIII*

Three hundred grams of diabetyl phthalate and 50 grams of glycerol mono-oleate were dissolved in 5,950 grams of perchlorethylene. A cellulose acetate netting curtain was wet out with the solution, dried, and ironed. When the stiffened curtain was hung, it draped nicely. On reaching an equilibrium of moisture saturation with respect to the surrounding atmosphere, the curtain was electro-conductive and did not balloon out or lose its original position of drape when subjected to friction.

It will be apparent from the foregoing examples that, in compounding the compositions of the invention, if the concentrations of the sizing agent and anti-static are controlled within the limits given, sizing agents and anti-static surface active agents of diverse chemical composition may be used together. In addition to the anti-static hygroscopic materials and electrolytes specifically illustrated, there may also be used, in admixture with the sizing agents, quaternary ammonium compounds such as paradiisobutyl-phenoxy ethoxyethyl dimethylbenzyl ammonium chloride and N-soya-N-ethyl morpholinium ethosulfate (supplied commercially as a 35% aqueous solution). Propylene glycol, glycerol mono-lauroate and mono-sulfonated glycerol compounds are also effective anti-static agents which are compatible with the sizing agents, in the concentrations stated, and may be used.

The conditions of the treatment, including the extent of dilution of the treating solution and the amount thereof picked up by the fibrous material may be varied, depending on the kind of fibrous material being treated, the relative humidity to which it is to be exposed, and the sizing and anti-static agents present in the treating solution or dispersion. In general, only comparatively small amounts of the sizing and anti-static agents are needed to accomplish the present objectives and it has been observed that treating solutions or dispersions containing between about 0.001% and about 0.050% of the anti-static agent, and about the same amount of sizing agent, are satisfactory. Greater or lesser amounts of these agents may be present in the treating composition, however, although generally speaking neither agent will be used in a concentration lower than about 0.001% by weight on the total solids weight.

The amount of the sizing and anti-static agents picked up by the fibrous material will depend on both the concentration thereof in the composition and the time of exposure of the fibrous material to the composition.

10  
5 On the basis of the weight of the fabric or other fibrous material being treated, it has been observed that the addition of from about 0.001% to 0.10% by weight of the treating solution or dispersion containing between 0.001% and 0.05% of each of the agents is usually sufficient to result, after drying, in an electro-conductive material carrying sufficient size to impart to it the desired stiffness. Here again the conditions may be varied and the addition of larger or smaller amounts of the treating composition to the fibrous material may be effected, when the fibrous material treated necessitates it.

This invention is particularly useful in the treatment of garments during or after dry-cleaning. The invention makes it possible to size the garment and render it electro-conductive, or to refreshen the garment by replenishing any size and anti-static agent removed during the dry-cleaning operation by a single treatment with a single homogeneous treating composition. Since only one treatment is required to achieve the dual purposes of sizing the garment and making it resistant to the accumulation of electrostatic charges, garments made of water-sensitive fabrics may even be treated with the less expensive aqueous solutions or dispersions of the compatible sizing and anti-static agents without being damaged by the treatment.

30  
15 The sizing agents and anti-static agents are defined herein in terms of minimum concentrations in which they are mutually compatible in the aqueous or non-aqueous vehicle. That range of concentrations is 0.001% to 40% by weight on the total solids weight of the composition. 20 However, while the homogeneous treating composition may comprise between 0.001% and 40%, each, or more generally, between 0.001% and 20% each, of the sizing and anti-static agents, the definition in terms of minimum compatible concentrations is not a limitation on the relative proportions of the two agents in the treating composition which may be higher for either or both in a given instance provided the requirement for compatibility and a homogeneous dispersion or solution is observed. A given sizing agent may be compatible in concentrations higher than stated with a selected anti-static agent. 25 Conversely, a given anti-static agent in a concentration higher than 40% may be compatible with the selected sizing agent. Or the sizing agent and anti-static agent may be mutually compatible in water or the dry-cleaning solvents in concentrations higher than 40% by weight. 30 Where higher concentrations of one or the other or both the sizing agent and anti-static agent result in homogeneous dispersions, the higher concentration may be used, if desired, and as will be apparent from a consideration of some of the foregoing examples, such as Example III, in which the calcium chloride is used in an amount of 80% by weight, on the total solids weight, as well as of Example IX below which illustrates still other compositions which are within the scope of this invention.

60

35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905

colloidal dispersions in which the dispersed particles fall within the colloidal range of sizes.

From the foregoing discussion, it will be seen that the present invention provides new compositions, and a new method, for simultaneously sizing fibrous materials and eliminating or materially reducing the tendency of such materials to become electrified when exposed to friction. It will also be understood that various changes and substitutions may be made in the compositions given herein without departing from the scope of this invention. Such variations, substitutions and modifications are contemplated as being within the scope of the invention as defined in the appended claims.

I claim:

1. A stable, concentrated, storable dispersion consisting essentially of water, from 5% to 40% by weight of gum arabic, and from 5% to 40% by weight of [alkyl (C<sub>9</sub> to C<sub>12</sub>)-butylmethyl]-trimethyl ammonium chloride, the dispersion being clear, homogeneous and essentially transparent and adapted to be diluted with water to provide a stable, clear, homogeneous essentially transparent treating bath for fabrics in which the fabrics are stiffened and simultaneously rendered electroconductive.

2. A stable, concentrated, storable dispersion consisting essentially of water, gum arabic, and [alkyl (C<sub>9</sub> to C<sub>12</sub>)-butylmethyl]trimethyl ammonium chloride, the dispersion being adapted to be diluted with water to provide a stable, homogeneous, essentially transparent treating bath for fabrics in which the fabrics are stiffened and simultaneously

rendered electroconductive, said gum arabic and alkyl ammonium chloride being present in the proportionate amounts, by weight, of about 10% and 1% of the concentrate, respectively.

References Cited in the file of this patent

UNITED STATES PATENTS

|           |                  |                |
|-----------|------------------|----------------|
| 1,421,700 | Lobeck           | July 4, 1922   |
| 2,054,257 | Hueter           | Sept. 15, 1936 |
| 2,086,544 | Dreyfus          | July 13, 1937  |
| 2,086,590 | Whitehead        | July 13, 1937  |
| 2,137,465 | Thackston        | Nov. 22, 1938  |
| 2,145,195 | Bauer et al.     | Jan. 24, 1939  |
| 2,149,046 | Finnell          | Feb. 28, 1939  |
| 2,197,930 | Jackson          | Apr. 23, 1940  |
| 2,277,788 | Shipp et al.     | Mar. 31, 1942  |
| 2,303,136 | Perkins          | Nov. 24, 1942  |
| 2,318,296 | Dickey           | May 4, 1945    |
| 2,381,020 | Wilkes et al.    | Aug. 7, 1945   |
| 2,419,281 | Noble            | Apr. 22, 1947  |
| 2,595,225 | Coffman          | May 6, 1952    |
| 2,626,877 | Carnes           | Jan. 27, 1953  |
| 2,649,143 | Simon et al.     | Aug. 18, 1953  |
| 2,651,583 | Horn et al.      | Sept. 8, 1953  |
| 2,658,843 | Brillhart        | Nov. 10, 1953  |
| 2,666,038 | Eisen            | Jan. 12, 1954  |
| 2,668,785 | Jefferson et al. | Feb. 9, 1954   |
| 2,694,021 | Griffin          | Nov. 9, 1954   |